

No. 831,914.

PATENTED SEPT. 25, 1906.

B. C. WHITE.  
MANUFACTURE OF GLASS SHEETS.  
APPLICATION FILED AUG. 12, 1905.

FIG.1.



FIG.2.



FIG.4.



FIG.3.



WITNESSES:

Robert Bradley.  
Francis Uman.

Bruce Clark White, INVENTOR  
by Christy and Christy, Atty's.

# UNITED STATES PATENT OFFICE.

BRUCE CLARK WHITE, OF MOSGROVE, PENNSYLVANIA.

## MANUFACTURE OF GLASS SHEETS.

No. 831,914.

Specification of Letters Patent.

Patented Sept. 25, 1906.

Application filed August 12, 1905. Serial No. 273,951.

*To all whom it may concern:*

Be it known that I, BRUCE CLARK WHITE, a citizen of the United States, residing at Mosgrove, in the county of Armstrong and State of Pennsylvania, have invented or discovered certain new and useful Improvements in the Manufacture of Glass Sheets, of which improvements the following is a specification.

10 In forming sheets of glass it is the common practice to pour the glass from a ladle onto a table or bed in front of a spreading-roll movable along the table or between suitably-arranged rolls. Although care is exercised to insure an even distribution of the glass along the front of the roll or between the rolls, it happens that a portion of the sheet at its front end will not have a width equal to that of the body of the sheet. In other words, 15 the sheet always begins with a point or narrow end and gradually widens out to the desired width. This irregularly-shaped front portion is useless and must be cut off, entailing considerable waste.

20 The invention described herein has for its object imparting to the body of glass to be rolled into a sheet a preliminary shape having one dimension—*i. e.*, the width of the sheet to be formed.

25 The invention is hereinafter described and claimed.

In the accompanying drawings, forming a part of this specification, Figure 1 is a plan view of a form of apparatus having rolls for shaping the sheet adapted for the practice of my invention. Fig. 2 is a sectional elevation on a plane indicated by the line II—II, Fig. 1. Fig. 3 is a perspective view of a form of apparatus in which the sheet is formed by the 30 conjoint action of a table and roll; and Fig. 4 is a view similar to Fig. 2, illustrating a modification.

In the practice of my invention the glass is taken from the furnace by a ladle or receptacle—such, for example, as that shown and described in an application filed by me August 12, 1905, Serial No. 273,952—formed in two parts or sections 1 and 2. The glass is scooped up by the closing of the sections and 35 is evenly distributed throughout the ladle or receptacle. The receptacle or ladle is made of a length equal or approximately equal to the width of sheet to be formed, and as the glass is evenly distributed in the receptacle 40 the glass will on the separation of the sec-

tions be evenly distributed between the rolls 3 in Figs. 1 and 2 or across the table 4 in front of the roll 5 in Fig. 3. While either of the constructions shown in the application Serial No. 273,952 may be used in the practice of my invention, it is preferred to use the construction in which the ladle-sections are maintained in parallelism. When the sheets are formed by the conjoint action of two rolls, as in Fig. 1, it is customary to pour the 45 glass into a hopper having its outlet in line with the opening between the rolls, and the glass will run between the rolls onto the movable supporting-table 4 in line with the first pouring, and as the ladle is moved along the 50 trough the sheet will finally attain full width. In the practice of my invention the ladle is forced in line with the opening between the rolls, and on the separation of the sections a stream of glass of a width equal to that of the 55 sheet to be formed will flow between the rolls. As the thickness of the stream of glass will be in accordance with the distance the sections are separated, it is apparent that the rolls may be used to only slightly reduce the 60 sheet flowing from the ladle and may, if desired, be entirely dispensed with, in which case the ladle would be suitably supported and the table or bed moved under it or the ladle moved along a stationary bed or table. 65

In the form of apparatus shown in Fig. 3 the table with the glass is moved to position in front of the roll and the sections opened, depositing on the table a mass of glass having a dimension parallel with the roll equal or approximately equal to the width of the sheet to be formed. With such an even distribution of glass in front of the roll the first part of the sheet formed by the movement of the roll will be of full width. 75

As is well known in the art, a portion of chilled or hardened glass incorporated in a plastic body after removal from the furnace will not be thoroughly remelted and will disfigure the article from such body of glass. 80 When glass is transferred by a tipping ladle to a shaping mechanism, the pouring from the ladle into the mechanism will inevitably cause the incorporation of any hardened particles on the ladle with the contents thereof. 85 In using my improved ladle the glass drops down without any turning over or stirring up into the shaping mechanism, so that any hardened particles, such as the thin film shown at *a* in Fig. 4, will pass in advance of the 90

95 glass at *b* in Fig. 4, and will not be incorporated in the sheet. 100

105

110

plastic glass between the rolls and the disfigurement caused thereby will be confined to a small portion of the front end of the sheet, which can be and generally is cut off. It will be observed that the bottom walls of my ladle conform approximately to the contour of the roll-surfaces, so that a portion of the body of glass is given a shape by the ladle approximately that which would be produced 10 by the parts or elements (e. g., the rolls) of the shaping mechanism first in contact with the glass.

As shown in Fig. 4, a feed-hopper may be used and the glass be deposited by the ladle 15 therein. The use of such hopper, which preferably corresponds as to length, width, and depth to the ladle, would not involve any undue agitation of the glass.

I claim herein as my invention—

20 1. As an improvement in the art of forming sheets of glass the method herein described, which consists in segregating a mass of glass, imparting to said mass of glass one of the dimensions of the sheet to be formed 25 and then reducing the mass of glass to sheet form.

2. As an improvement in the art of forming sheets of glass the method herein described, which consists in segregating a mass 30 of glass, imparting to such segregated mass of glass a dimension equal or approximately equal to the width of the desired sheet, feeding such shaped mass to shaping elements or

parts and then reducing the glass to the desired thickness.

3. As an improvement in the art of forming sheets of glass the method herein described which consists in giving to a segregated mass of glass while removing it from the furnace, a dimension equal or approximately equal to one of the dimensions of the sheet to be formed, and then reducing the glass to sheet form.

4. As an improvement in the art of forming sheets of glass the method herein described which consists in giving to a segregated mass of glass, prior to feeding it to the sheet-forming mechanism, a dimension equal or approximately equal to one of the dimensions of the sheet to be formed, and reducing 45 the glass to the desired thickness.

5. As an improvement in the art of forming sheets of glass, the method herein described, which consists in detaching and removing a mass of glass from a furnace, and 55 imparting to such removed or detached mass a shape or configuration similar or substantially similar to that of the parts or elements first operative on the glass in reducing it to sheet form.

In testimony whereof I have hereunto set my hand.

BRUCE CLARK WHITE.

Witnesses:

MINNIE C. JONES,  
FRANCES VERNAN.